

# UNITED STATES PATENT OFFICE.

ROLAND B. RESPESSE, OF NEW YORK, N. Y.

## LEATHER SUBSTITUTE AND PROCESS FOR MAKING THE SAME.

1,276,113.

Specification of Letters Patent. Patented Aug. 20, 1918.

No Drawing.

Application filed November 26, 1917. Serial No. 203,932.

*To all whom it may concern:*

Be it known that I, ROLAND B. RESPESSE, a citizen of the United States, and resident of the borough of Manhattan, city of New York, in the county of New York and State of New York, have invented certain new and useful Improvements in Leather Substitutes and Processes for Making the Same, of which the following is a specification.

10 This invention relates to leather substitute and the process for making the same. The steps and products of this invention are an improvement of the steps and product described and claimed in my patent application for rubber fabrics and molded rubber and processes for making the same, filed in the United States Patent Office on or about July 13th, 1917, Serial Number 180,428.

One of the objects of the present invention 20 comprises the production and process of making a strong, pliable, unwoven material of matted fibers formed into sheets or mats having the appearance of undressed split leather. The product may be finished and 25 grained to resemble leather, in the same manner that leather is usually finished. The process primarily consists in taking suitable vegetable, animal or mineral fibers such as hemp, flax, cotton, jute, ramie, wood-fiber, 30 wool, hair, asbestos or the like and form therewith sheets or mats, with the fibers thereof located in any and all directions.

The fibers are preferably located in place by garnetting, carding or other suitable 35 machines. The sheets or mats are passed between rollers and compressed, after which they are saturated with a binding agent, that causes the fibers to adhere to each other after being dried. After the sheets or mats 40 are dried, they are again passed between rollers and compressed, and a strong flexible sheet of material is produced resembling split leather. The sheets or mats are next surfaced with a suitable dressing, passed between heated graining rolls, which embosses 45 designs on the sheets or mats and produces a finished product having the appearance of grained leather.

One exemplification of the invention comprises the following:

Raw cotton and ramie are mixed and formed into sheets or mats by means of garnetting, carding or other suitable machinery. The formed sheets or mats of cotton 55 and ramie are then passed between rollers and compressed. The compressed sheets are

then saturated with a binding agent, which may consist of the following: Rubber gum dissolved in naphtha or benzol to make about a three percentum solution. To one 60 gallon of this rubber solution is added one third ounce of balata which has been reduced to a liquid by a suitable solvent, one sixth ounce fish glue, one third ounce silicate of soda, one sixth ounce of sulfur and 65 one sixth ounce of linseed oil. The proportions of the ingredients of the binding agent may be varied to produce either a heavy coarse fabric or a soft flexible material. Next the sheets or mats are dried and again 70 passed between rollers and compressed, which forms a sheet or mat resembling split leather. The sheets or mats are then surfaced with a suitable dressing of any desired color. The sheets or mats are next passed 75 through heated graining rollers and thereby embossed and designs formed thereon, which produces a finished product having the appearance of finished leather. The raw fiber before being formed into sheets or mats may 80 be treated with a dyeing agent to obtain the color required for the finished product. The binding agent may also have introduced therein a coloring agent.

Having described my invention, what I desire to secure by Letters Patent and claim is:

1. The herein described process of making a leather substitute consisting in forming a matted fiber sheet, compressing the said sheet and saturating it with a binding agent 90 composed of rubber, balata, fish glue, silicate of soda, sulfur and linseed oil, drying the sheet and compressing it.

2. The herein described process of making a leather substitute consisting in forming 95 a matted fiber sheet, compressing the sheet, saturating it with a binding solution composed of rubber, balata, fish glue, silicate of soda, sulfur and linseed oil, drying the sheet, compressing it, surfacing the sheet 100 with a suitable dressing and passing it between heated graining rollers.

3. The herein described process of making a leather substitute consisting in forming a dyed matted fiber sheet, compressing the 105 sheet, saturating it with a binding solution composed of rubber, balata, fish glue, silicate of soda, sulfur and linseed oil, drying the sheet, compressing it, surfacing the sheet with a dressing and passing it between 110 heated graining rollers.

4. The herein described process of mak-

ing a leather substitute consisting in forming a sheet of fibers, compressing the sheet, saturating it with a binding solution composed of rubber, balata, fish glue, silicate 5 of soda, sulfur, linseed oil, and a coloring agent, drying the sheet, compressing it, surfacing the sheet with a dressing and passing it between heated graining rollers.

5. A leather substitute comprising matted 10 fibers, and a binding agent comprising rub-

ber, naphtha, balata, fish glue, silicate of soda, sulfur and linseed oil.

Signed at the borough of Manhattan, city of New York, in the county of New York and State of New York, this 25th day of 15 November, A. D. 1917.

ROLAND B. RESPRESS.

Witnesses:

A. A. DE BONNEVILLE,  
A. W. BAKER.